

M. E. HOLMES,  
BATTERY DEPOLARIZER.  
APPLICATION FILED DEC. 13, 1913.

1,218,772.

Patented Mar. 13, 1917.



*WITNESSES.*

WITNESSES  
L. Raufer.  
H. G. Grover

INVENTOR  
MAJOR E. HOLMES

BY Ira Adams

**ATTORNEY**

# UNITED STATES PATENT OFFICE

MAJOR E. HOLMES, OF LAKewood, OHIO, ASSIGNOR TO NATIONAL CARBON COMPANY,  
OF CLEVELAND, OHIO, A CORPORATION OF NEW JERSEY.

## BATTERY-DEPOLARIZER.

1,218,772.

Specification of Letters Patent. Patented Mar. 13, 1917.

Application filed December 13, 1913. Serial No. 806,356.

To all whom it may concern:

Be it known that I, MAJOR E. HOLMES, a citizen of the United States, residing at Lakewood, in the county of Cuyahoga and State of Ohio, have invented a certain new and useful Improvement in Battery-Depolarizers, of which the following is a full, clear, and exact description.

This invention relates to the preparation of battery depolarizers and more particularly to manganese compounds for such use in dry cells. Most dry cells use manganese depolarizers in the form of the natural oxid  $MnO_2$  which is commonly known as pyrolusite. The natural manganese peroxid is not, however, obtained in a pure state and does not form a perfectly satisfactory depolarizer. This is due partially to its low peroxid content, but principally to the difficulty with which the oxygen is given off, and to the impurities, which not only decrease the available oxygen but are actually harmful to the depolarizing action. To prevent these difficulties various artificially prepared manganese compounds have been proposed. Most of these artificial depolarizers are more or less satisfactory because the impurities have some depolarizing value, but the chemicals required for their preparation are so expensive that it is impracticable to use the product in a dry cell, except in some instances in the so-called "midget" cell. In such cells an expensive depolarizer may be used because the quantity required is very small and the best materials are necessary to secure a serviceable battery built up in such a limited space. The cost, however, prevents its use in the larger sizes of dry cells.

One of the objects of my invention is to prepare an artificial battery depolarizer of increased depolarizing efficiency.

Another object is to decrease the cost of production of an artificial depolarizer, by using cheap materials and by utilizing the materials formed in the reaction of the process.

Additional objects will appear in the specification and drawing, in which:

The single figure is a diagrammatic view of a form of apparatus for carrying out the process.

It will be understood, however, that the apparatus shown in the drawing is not the

only form which could be used and the broader aspect of the invention will be particularly set forth in the claims. In my co-pending application, Serial No. 794,360, filed October 10, 1913, I have referred to a process of making colloidal manganese peroxid in which the method is somewhat similar to the process herein described. This process is also suitable for the manufacture of either crystalloidal or colloidal manganese peroxid by regulating certain conditions under which the reaction occurs.

In the drawing 1 represents an electrolytic cell of the well known Townsend type for the manufacture of sodium hydroxid and chlorin gas by the electrolysis of a salt solution.

Other electrolytic cells producing sodium or other hydroxids and chlorin simultaneously would also be suitable. This cell consists of an iron receptacle 2 open at the top and bottom. Cathode plates 3 made of perforated iron sheets are fastened within the receptacle between the top and bottom so as to form three chambers 4, 5 and 6. The chambers 4 and 5 are located between the walls of the receptacle 2 and each of the cathode plates 3, and the chamber 6 is located between the two cathode plates 3. The top and bottom openings of the receptacle are closed by means of a suitable insulating cover 7 and base 8. Inside the cathodes 3 is placed a diaphragm 9 of woven asbestos cloth having the pores filled for example with iron oxid, asbestos fiber and colloidal iron hydroxid. Through the cover 7, an anode 10 of graphite is inserted in the chamber 6. In the top of the cover 7, an opening 11 controlled by a valve 12 is provided for the admission of salt solution. A funnel or reservoir 13 may be used for the addition of the solution to be electrolyzed, and an opening 14 is left in the cover for the removal of the chlorin formed.

The electrolyte, namely, sodium or other chlorid solution, is admitted to the chamber 6 through the opening 11 and slowly permeates through the diaphragm 9. The exterior chambers 4 and 5 have openings 15 for removing, and collecting apparatus 15' for saving, the hydrogen gas formed by the reaction. These chambers 4 and 5 contain kerosene which takes no part in the reaction and serves for settling the

heavier sodium hydroxid formed. At the bottom of the chambers 4 and 5, depending on channels or grooves 16 are arranged with outlet pipes 17 for the removal of the sodium hydroxid which percolates through the diaphragm. Since chlorin and sodium hydroxid are two of the chemicals used, manganous chlorid being the other, the use of such a cell is obviously very advantageous in my process.

Below the electrolytic cell is a reservoir 17' for collection of the sodium hydroxid which is removed therefrom as desired at the base through an outlet 18 controlled by a valve 19. A reaction chamber 20 into which the chemicals for producing the reaction are admitted is arranged below the receptacle 17'. Another receptacle 21 having a controlling valve 22 contains the manganous chlorid used for the reaction and is also conveniently located above the reaction chamber.

Chlorin formed during the electrolysis in the cell is conducted through a pipe 23 from the electrolytic cell into the reaction chamber 20. To facilitate the circulation of the gas, a fan or other device 24 may be inserted in the pipe and a controlling valve 25 may also be used to control the flow of gas.

The material formed by the interaction of chemicals in the reaction chamber is removed at the bottom through a pipe 24' and valve 25' and conveniently collected in a settling chamber 26. The supernatant liquid may be removed from the chamber by means of a tube 27 and returned to the electrolytic cell to be electrolyzed again. To raise the supernatant liquid to the electrolytic cell 1, a pump 28 may be used and a valve 29 will regulate the removal. The supernatant liquid may also be removed from the settling chamber, through a pipe 30 having a valve 31 in its circuit, by means of the pump 28 already mentioned. It may then be conducted into the electrolytic cell through the pipe 32.

When a source of E. M. F. is applied to the terminals of the electrolytic cell containing the electrolyte of salt solution, chlorin will be formed at the graphite anode 10 and collect in the chamber 6. The sodium ion traveling toward the cathode will react, upon being discharged, with the water present in the salt solution, to form sodium hydroxid and at the same time liberate hydrogen. The sodium hydroxid together with the salt solution which percolates through the diaphragm will settle in the grooves 16 of the chambers 4 and 5, because it is considerably heavier than the kerosene in the chambers. The hydrogen will be removed through the vents 15 and be collected in the reservoir 15'. The action of the electrolytic cell need not be further described as it is old and well known in the art, but its use in connection with this process is especially advantageous

because the products are so particularly suitable that the entire process is rendered very economical.

The sodium hydroxid solution collecting in the grooves 16 containing in addition considerable salt in solution is withdrawn into the receptacle 17' as it is formed and later admitted as required into the reaction chamber 20 containing manganous chlorid, which is withdrawn from the reservoir 21 by opening the valve 22. Since manganous chlorid is one of the least expensive salts of manganese its utilization is a further step toward obtaining an inexpensive product. Into this solution, containing manganous chlorid, sodium chlorid and sodium hydroxid, the chlorin gas generated in the electrolytic cell is passed continuously through the pipe 23 by fan 24. In order to thoroughly submit the mixture to the gas it is necessary to stir or shake the solutions thoroughly. For this purpose a stirring device 33 driven by a pulley 34 and belt 35 may be used advantageously. Sodium hydroxid is conducted either continuously or from time to time into the reaction chamber in such quantities as to keep the mixture in the reaction chamber approximately neutral in reaction. If the mixture is maintained strongly alkaline, colloidal material will be formed as set forth in the co-pending application referred to.

The reaction between the  $\text{NaOH}$  and  $\text{MnCl}_2$  forms manganous hydroxid which is then oxidized to a manganic compound, such as an oxid or manganite by the action of the chlorin. The oxidizing action of chlorin is due to the formation of hydrochloric acid and nascent oxygen when the chlorin gas reacts on the water present. The sodium hydroxid present will unite with the hydrochloric acid mentioned to form sodium chlorid. This salt, as well as that present in the hydroxid solution, does not enter into the reaction, occurring in the chamber 20. In forming the manganic compound from the manganous hydroxid many intermediate compounds are formed before the  $\text{Mn}(\text{OH})_2$  is completely oxidized, so that no equation would express the reaction completely.

From the above reaction it will be evident that sodium chlorid is reformed substantially equivalent to the amount consumed because the sodium hydroxid combines with the  $\text{MnCl}_2$  and  $\text{HCl}$  to form this salt. As the depolarizer is precipitated, the sodium chlorid solution may be withdrawn if desired and returned to the electrolytic cell through the pipes 30 and 32 by the pump 28. As salt is relatively inexpensive, however, the solution need not necessarily be returned to the cell, although such economy is desirable.

To complete the reaction and completely oxidize the manganous compound, chlorin is passed through the solutions in the closed re-

action chamber for a considerable time. The solution must also be stirred or shaken occasionally in order to subject all of the mixture to the action of the chlorin. From 3 to 5 6 hours has been found to be necessary to obtain a good product under these conditions. During this time the sodium hydroxid is added from time to time so as to keep the mixture approximately neutral and 10 thus neutralize the hydrochloric acid formed which would tend to dissolve the manganese oxids if the solution became strongly acid. By the use of a strongly alkaline solution, I obtain more or less colloidal manganese 15 peroxid intermixed with the crystalloidal form and my invention is intended to include the manufacture of such material by this process. All of the manganese chlorid is preferably introduced into the reaction 20 chamber at the same time, but if desired may be added from time to time. After the reaction is complete, the solution and precipitate are removed to the settling chamber and the supernatant liquid may be returned to 25 the electrolytic cell as previously described.

The quantity of sodium hydroxid required for the reaction is considerably more than would be expected because much of it is consumed in preventing the solution becoming 30 too strongly acid on account of the hydrochloric acid formed as an intermediate product. Considerable chlorin is formed in excess of the amount required for the reaction. This escapes through the liquid and may be 35 saved by conducting through a pipe 36 into collector 37. This chlorin may be utilized in any manner, as for instance, to make bleaching powder by passing the gas through calcium oxide or to make depolarizer by passing the gas through a mixture of solutions of a manganese salt and calcium hydroxid or other hydroxids.

It will be understood that although the sodium hydroxid and chlorin required for 40 the reaction are preferably formed in the electrolytic cell that this need not necessarily be the case as these materials may be obtained in other ways. The broad feature of the invention is the use of chlorin 45 gas to precipitate a depolarizer from a solution of a salt of manganese. By such precipitation a very efficient depolarizer is obtained which has a high oxygen content 50 which is readily given off when used in a dry cell. Its specific gravity and cheapness 55 also satisfy all requirements for a good depolarizing material.

The composition of the material will vary somewhat depending upon certain conditions such as the length of time the solutions 60 are submitted to the action of the chlorin gas.

If the supernatant liquid is not to be used again in the electrolytic cell, other manganese salts may be used such as  $MnSO_4$  for 65 instance.

Having described my invention, what I claim is:

1. The method of making a battery depolarizer which consists of precipitating a 70 manganese hydroxid from a manganese compound and oxidizing the hydroxid with chlorin.

2. The method of making a battery depolarizer which consists in precipitating a 75 manganese hydroxid from a solution of manganese chlorid by means of a hydroxid and oxidizing it with chlorin.

3. The method of making a battery depolarizer which consists in precipitating a 80 manganese hydroxid from a solution of a manganese salt, gradually admitting chlorin to oxidize the manganese hydroxid and simultaneously admitting a hydroxid to neutralize the acid formed by the said oxidation.

4. The method of making a battery depolarizer which consists in electrolyzing a chlorid to form a hydroxid and chlorin gas, and treating a manganese compound with 90 the hydroxid and the chlorin.

5. The method of making a battery depolarizer which consists in forming a hydroxid and chlorin gas by electrolysis of a chlorid solution, precipitating a manganese 95 hydroxid from a manganese salt by means of the first mentioned hydroxid and oxidizing the manganese hydroxid by treatment with the chlorin.

6. The method of making a battery depolarizer which consists in electrolyzing a chlorid solution to form a hydroxid and chlorin gas and admitting the hydroxid and chlorin gradually into a solution of manganese chlorid to precipitate a manganic 105 compound.

7. The method of making a battery depolarizer which consists in electrolyzing a chlorid solution to form a hydroxid and chlorin gas, admitting the hydroxid to a 110 solution of a manganese salt to precipitate a manganese hydroxid, admitting the chlorin to the mixture to oxidize the manganese hydroxid to a manganic compound, and adding more hydroxid from time to time to neutralize the hydrochloric acid formed by the 115 said oxidation.

In testimony whereof, I hereunto affix my signature in the presence of witnesses.

MAJOR E. HOLMES.

Witnesses:

IRA J. ADAMS,  
H. G. GROVER.